

May 20, 1952

G. E. RICKNER ET AL

2,597,182

SURFACING GLASS SHEETS OR PLATES

Filed March 31, 1949



Fig. 1



Fig. 2



Fig. 3



Fig. 4

INVENTORS

George E. Rickner and  
BY Oscar R. Koenig  
Nobbe G. Swope

ATTORNEYS

## UNITED STATES PATENT OFFICE

2,597,182

## SURFACING GLASS SHEETS OR PLATES

George E. Rickner and Oscar F. Koenig, Ottawa,  
Ill., assignors to Libbey-Owens-Ford Glass  
Company, Toledo, Ohio, a corporation of Ohio

Application March 31, 1949, Serial No. 84,674

14 Claims. (Cl. 51—283)

1

The present invention relates broadly to the surfacing of glass sheets or plates, and more particularly to a novel smoothing treatment, between the customary grinding and polishing steps.

Briefly stated, the invention is based on the discovery that surprisingly better and faster surfacing of glass blanks can be accomplished by smoothing or preliminarily polishing the blanks, after grinding and before polishing, with a mixture of rouge and pumice rubbed over the glass blanks by relatively soft, resilient runners or tools.

While not restricted to such use, the present invention has proved to be of outstanding value when employed in the socalled continuous method of grinding and polishing plate glass blanks. In this method, as now quite widely practiced, a plurality of rough glass blanks are mounted upon a series of cars or tables, arranged in end to end relation and movable continuously along a definite predetermined path to carry the glass blanks first through a grinding and then through a polishing area. In the grinding area the blanks are subjected to the abrasive action of sand of progressively decreasing coarseness, under heavy iron runners, and in the polishing area the ground surfaces of the blanks are polished with rouge under felt pads.

This is the method that has been generally used by the company to which this application has been assigned for many years. Now, however, we have discovered that better results can be had, that the surfacing operation can be better controlled, and that higher production speed can be attained, by subjecting the glass to the special smoothing operation of this invention while it is passing between the grinding and polishing areas.

In fact, where this invention has been incorporated in a grinding and polishing line, we have increased the speed of the line, in actual commercial production from 110 to 140 inches per minute with remarkably good results in surface finish of the glass; and this increase in line speed represents an increased production of between 25 and 30% on this line.

We do not claim to be the first to suggest the broad idea of smoothing or preliminarily polishing glass blanks between the conventional grinding and polishing steps, because this has been suggested before. And various types of abrasives such as extremely fine or waste sand, garnet, fine pumice, etc., applied with tools of different types, have also been suggested for the purpose.

2

But none of these procedures that we have tried have worked to our satisfaction, and with none of them have we been able to accomplish the results which we have attained with our present smoothing technique.

It is therefore an aim of this invention to provide a commercially successful smoothing technique which, when employed between conventional grinding and polishing steps, will not only improve surface quality of the glass, but will also permit it to be surfaced in a shorter length of time and/or, in the case of a continuous process, with fewer tools.

Another object is the provision of a smoothing method of this character in which a mixture of rouge and pumice is employed as the abrasive.

Another object is to provide a method of the above character in which a special mixture of rouge, pumice and copperas in water is rubbed over the ground glass surfaces by relatively soft, compressible tools.

Still another object is the provision of a special mixture for the above purpose in which pumice of a particular particle size is mixed with a definite proportion of rouge in water and sufficient copperas added to give a predetermined reading on the Baumé scale.

Other objects and advantages of the invention will become more apparent during the course of the following description, when taken in connection with the accompanying drawings.

In the drawings, wherein like numerals are employed to designate like parts throughout the same;

35 Fig. 1 is a fragmentary, diagrammatic, plan view of a continuous grinding and polishing line showing our smoothing apparatus in position;

Fig. 2 is a section taken substantially on the line 2—2 in Fig. 1, showing the construction of a 40 preferred type of smoothing tool;

Fig. 3 is a view similar to Fig. 2, showing a modified type of smoothing tool; and

Fig. 4 is a bottom view of the tool shown in Fig. 3.

45 Referring now more particularly to the drawings, there has been illustrated in Fig. 1 a well known type of continuous grinding and polishing line, indicated generally by the numeral 10. The exit end of the grinding area is indicated at the 50 left of this figure at 11, and the entrance end of the polishing area is indicated at the right at 12.

In the line, a series of tables 13 are bolted together to form a continuous glass supporting surface on which blanks 14 are bedded in a layer of

plaster of Paris 15. The tables 13 are continuously moved in the direction of the arrows 16 to carry the blanks first beneath a series of iron grinding runners 17, beneath which sand of progressively increasing fineness is fed, and then beneath a series of polishing heads 18, which are supplied with rouge in any well known manner.

Suitable cleaning means, shown diagrammatically at 19, are provided at the end of the grinding area to remove all traces of grinding sand from the glass surfaces before they move toward the polishing area.

In practicing our invention, we interpose, in the area 20, between the grinding and polishing areas, a plurality of smoothing runners or tools 21. These tools may be made in various sizes and shapes and can be arranged in any one of a number of different ways. However, in actual practice, we have found that four sets of three overlapping tools each, and with the tools themselves elliptical in shape, give very good results. The individual tools, located as shown in Fig. 1, are rotated in the directions of the arrows, and the sets of tools may be reciprocated transversely of the glass on the line if desired.

Satisfactory results have been obtained when the individual smoothing tools are rotated at any speed between 40 and 100 R. P. M., but best results seem to be had at speeds of around 55 R. P. M.

Practically any construction of smoothing tool can be employed with our invention so long as the glass contacting surface of the tool is compressible, and not too soft. For example, either felt or rubber tools can be used. However, we prefer a felt tool of the general character shown in Fig. 2, and which comprises a metal plate 22 carried at the end of a spindle 23 and having a wooden plate 24 affixed to and covering its lower face. Strips of felt, rubber or the like 25, arranged in face to face relation to one another and extending across the face of the plate 24, are secured to this plate by nailing, adhesively, or in any other desired and permanent manner. The advantage of this particular construction of tool seems to lie in the fact that the fissures or cracks 26 between the adjacent strips assist in distributing the rouge and pumice mixture uniformly over the smoothing face 27 of the tool.

An alternate form of tool that has been used with good results is shown in Figs. 3 and 4, and comprises a plate 28 carried at the end of a spindle 29 and having a thick sheet or pad of felt or similar compressible material 30 covering, and preferably cemented to, its lower face 31. The lower, or glass contacting face of the felt pad 30 is preferably provided with grooves 32, leading from a central opening 33 to the edges of the tool, to distribute the rouge and pumice mixture over the smoothing face of the tool. And this may be further facilitated by bays 34 also leading out from the central opening. In the case of either of the tools shown in Figs. 2 and 3, the mixture of rouge and pumice may be supplied to the tool through a passageway 35 in the spindles 23 and 29 or it may be deposited on the glass in the path of travel of the tool.

A pointed out above, we have found that an extremely efficient smoothing action, which influences and improves the entire surfacing operation to a remarkable degree, can be obtained by treating the glass, between the grinding and polishing areas, with a mixture of pumice and rouge rubbed over the ground glass surfaces with compressible tools of the general character just described.

Surprisingly enough, we have also discovered that a coarser grade of pumice than has heretofore been considered to be adapted to finishing glass surfaces gives the best results in the rouge and pumice mixture. Specifically, grades between ".0%" and ".0½ special" should be used for proper smoothing, because grades above ".0%" are found to be too coarse, while grades below ".0½ special" are too fine.

The term ".0%" is used by pumice manufacturers to indicate a grade of pumice consisting of substantially the particle sizes, in substantially the proportions, shown in the column at the left of the table below; and ".0½ special" is used to indicate a grade of pumice consisting of substantially the particle sizes, in substantially the proportions, shown in the extreme right column in the table:

| Grade of Pumice..... | Per Cent Between Sieves |       |       |             |
|----------------------|-------------------------|-------|-------|-------------|
|                      | .0%                     | X     | Y     | .0½ Special |
| 25 Sieve No.:        |                         |       |       |             |
| 42.....              |                         | N     | N     |             |
| 48.....              | N                       | 12P±  | 5P    | N           |
| 60.....              | 4P                      | FP    | FP    | FP          |
| 65.....              |                         | 2.7   | T     | 0.1         |
| 80.....              | 0.1                     | 9.6   | 0.4   | 1.1         |
| 100.....             | 14.0                    | 17.4  | 9.8   | 15.3        |
| 150.....             | 42.7                    | 26.1  | 30.0  | 39.8        |
| 200.....             | 30.8                    | 27.5  | 35.0  | 23.3        |
| 250.....             | 2.9                     | 8.2   | 11.1  | 5.3         |
| +325.....            | 5.5                     | 5.5   | 7.5   | 14.7        |
| -326.....            | 4.0                     | 3.0   | 6.2   | 0.4         |
| Total.....           | 100.0                   | 100.0 | 100.0 | 100.0       |

N=None.  
P=Pieces (number indicated).  
VFP=50 to 100 pieces.  
FP=100 to 200 pieces.  
T=About 300 pieces.  
Recorded to nearest .1%.

Grades X and Y in the table are grades of pumice, falling between ".0%" and ".0½ special," that were made up especially for this purpose. Any of these four grades of pumice, or any other grade falling between the outside limits given above, will operate satisfactorily. However, we prefer ".0%" and "X," and recommend these grades for use in regular commercial production.

After selecting the proper grade of pumice, the pumice is mixed with rouge, preferably in the ratio of 165 pounds of pumice to 50 pounds of rouge in 600 gallons of water or other suitable liquid, which has previously been made up with an amount of copperas, or ferrous sulphate ( $FeSO_4$ ), to form "acid" and to give a reading of 0.6° on the Baumé scale for heavy liquids.

Some variations in the proportions of the ingredients in the rouge and pumice mixture are permissible while still maintaining its effectiveness. However, we have found that a range between 125 and 165 pounds of pumice to 50 pounds of rouge is best for most effective smoothing. Within this range the amount of work done will increase by approximately 1 micro inch for each additional 20 pounds of pumice in the mixture.

On the other hand, a mixture containing much more than 165 pounds of pumice to 50 pounds of rouge does not flow as satisfactorily, and a mixture containing less than 100 pounds of pumice, to 50 pounds of rouge, will accomplish only slightly more work than will rouge or pumice alone.

Similarly, we prefer to use approximately 50 pounds of rouge to 165 pounds of pumice in the mixture, although anywhere in the range of 40 to 60 pounds of rouge to 165 pounds of pumice gives

good results. Even a slightly wider range can be used, but we seem to lose the amount of work the pumice can do in the mixture when the amount of rouge is increased much above 60 pounds, and amounts of rouge outside of a range of 25 to 75 pounds to 165 pounds of pumice will not give results that are commercially satisfactory for our purpose, although some good effects will be noted all the way down the scale.

In other words, while there are definite proportions of rouge and pumice that should be adhered to in order to obtain the greatly improved results we have noted from our novel smoothing technique, a mixture of rouge and pumice in any proportion will give better results than either rouge or pumice alone. Thus, the use of rouge alone in the smoothing area will give no different results than are obtained in the polishing area 12, and pumice when used without rouge is a thin watery mix which runs away and will not adhere effectively to the smoothing tools.

As indicated above, we use about 600 gallons of water for the rouge and pumice mixture, but this can be varied to meet actual working conditions, the important thing being to keep a concentration, that is not too great to clog the pipes, nor so dilute as to wash out the smoothing material from the tools before it can do the required work.

The water should contain copperas (ferrous sulphate) and we prefer an amount to give a reading for the water and copperas mixture of 0.6° on the Baumé scale for heavy liquids. The presence of the copperas is important in the mixture because it acts to hold the rouge in suspension in the water and to disperse the rouge particles, causing them to float through the liquid without sticking together.

Moreover, the rouge and copperas in the mixture combine to provide a proper carrying liquid of the specific gravity necessary to suspend the pumice particles, and provides a bonding agent tending to effectively hold the pumice in working engagement with the smoothing tools.

Although we prefer an amount of copperas to give a reading of 0.6 on the Baumé scale, an amount that will give a reading within the range of 0.4° to 1.0° Baumé can be used. Below the minimum, however, the rouge will not be properly suspended in and dispersed through the liquid, while an amount of copperas above the maximum will cause the block to harden to a point where it will run over the glass with too little smoothing effect.

In this connection, and particularly when felt tools are used, it is extremely important to control the amount of copperas used, and to clean the felts frequently in order to maintain them in a sufficiently soft condition to give proper smoothing.

It is also desirable to provide a cleaning means at the end of the smoothing area 20, that is similar to the cleaning means 19, to remove the smoothing materials from the surface of the glass before it passes into the polishing area 12.

In fact, it is to be understood that the forms of the invention herewith shown and described are to be taken as illustrative embodiments only of the same, and that various changes in the shape, size and arrangement of parts may be resorted to without departing from the spirit of the invention or the scope of the subjoined claims.

We claim:

1. In a method of surfacing glass sheets or plates in which a surface of such a plate is first

ground with sand of progressively increasing fineness applied with hard tools and then polished with rouge under relatively soft tools, the step of smoothing said surface after grinding and before polishing by rubbing a mixture of rouge and pumice with copperas in a liquid carrier over said surface with compressible tools.

2. In a method of surfacing glass sheets or plates in which a surface of such a plate is first 10 ground with sand of progressively increasing fineness applied with hard tools and then polished with rouge under relatively soft tools, the step of smoothing said surface after grinding and before polishing by rubbing a mixture of 15 rouge and pumice in proportions of between 25 and 82.5 parts of rouge by weight to 165 parts of pumice by weight with copperas in a liquid carrier over said surface with compressible tools.

3. In a method of surfacing glass sheets or plates in which a surface of such a plate is first 20 grounded with sand of progressively increasing fineness applied with hard tools and then polished with rouge under relatively soft tools, the step of smoothing said surface after grinding and before polishing by rubbing a mixture of 25 rouge and pumice in proportions of between 25 and 82.5 parts of rouge by weight to 165 parts of pumice of a grade between ".034" and ".012 special" by weight with copperas in a liquid carrier over said surface with compressible tools.

4. In a method of surfacing glass sheets or plates or the like in which a surface of such a plate is first ground with sand of progressively increasing fineness applied with hard tools and then polished with rouge under relatively soft tools, the step of smoothing said surface after grinding and before polishing by rubbing a mixture of 35 rouge and pumice in proportions of between 25 and 82.5 parts of rouge by weight to 165 parts of pumice of a grade between ".034" and ".012 special" by weight in water to which copperas has been added to give a reading of between 0.4° to 1.0° on the Baumé scale over said surface with compressible tools.

5. In a method of surfacing glass sheets or plates or the like in which a surface of such a plate is first ground with sand of progressively increasing fineness applied with hard tools and then polished with rouge under relatively soft tools, the step of smoothing said surface after 45 grinding and before polishing by rubbing a mixture of rouge and pumice in proportions of between 40 and 60 parts of rouge by weight to 165 parts of pumice of a grade between ".034" and ".012 special" by weight in water to which copperas has been added to give a reading of between 0.4° and 1.0° on the Baumé scale over said surface with compressible tools.

6. In a method of surfacing glass sheets or plates or the like in which a surface of such a plate is first ground with sand of progressively increasing fineness applied with hard tools and then polished with rouge under relatively soft tools, the step of smoothing said surface after 50 grinding and before polishing by rubbing a mixture of rouge and pumice in proportions of 50 parts of rouge by weight to between 125 and 165 parts of pumice of a grade between ".034" and ".012 special" by weight in water to which copperas has been added to give a reading of between 0.4° and 1.0° on the Baumé scale over said surface with compressible tools.

7. In a method of surfacing glass sheets or plates or the like in which a surface of such a plate is first ground with sand of progressively

increasing fineness applied with hard tools and then polished with rouge under relatively soft tools, the step of smoothing said surface after grinding and before polishing by rubbing a mixture of rouge and pumice in proportions of between 40 and 66 parts of rouge by weight to 165 parts of pumice of a grade between ".03/4" and ".0 1/2 special" by weight in water to which copperas has been added to give a reading of between 0.4° and 1.0° on the Baumé scale over said surface with compressible tools.

8. In a method of surfacing glass sheets or plates or the like in which a surface of such a plate is first ground with sand of progressively increasing fineness applied with hard tools and then polished with rouge under relatively soft tools, the step of smoothing said surface after grinding and before polishing by rubbing a mixture of rouge and pumice in proportions of between 40 and 66 parts of rouge by weight to 165 parts of pumice of a grade having substantially the following per cent of particles of the indicated fineness between sieves:

| Sieve No. | Per Cent Between Sieves |
|-----------|-------------------------|
| 42        | -----                   |
| 48        | N                       |
| 60        | 4P                      |
| 65        | VFP                     |
| 80        | 0.1                     |
| 100       | 14.0                    |
| 150       | 42.7                    |
| 200       | 30.8                    |
| 250       | 2.9                     |
| +325      | 5.5                     |
| -325      | 4.0                     |

by weight in water to which copperas has been added to give a reading of between 0.4° and 1.0° on the Baumé scale over said surfaces with compressible tools.

9. In a method of surfacing glass sheets or plates or the like in which a surface of such a plate is first ground with sand of progressively increasing fineness applied with hard tools and then polished with rouge under relatively soft tools, the step of smoothing said surface after grinding and before polishing by rubbing a mixture of rouge and pumice in proportions of between 40 and 66 parts of rouge by weight to 165 parts of pumice of a grade having substantially the following per cent of particles of the indicated fineness between sieves:

| Sieve No. | Per Cent Between Sieves |
|-----------|-------------------------|
| 42        | N                       |
| 48        | 12P+                    |
| 60        | FP                      |
| 65        | 2.7                     |
| 80        | 9.6                     |
| 100       | 17.4                    |
| 150       | 26.1                    |
| 200       | 27.5                    |
| 250       | 8.2                     |
| +325      | 5.5                     |
| -325      | 3.0                     |

by weight in water to which copperas has been added to give a reading of between 0.4° and 1.0° on the Baumé scale over said surfaces with compressible tools.

10. In a method of surfacing glass sheets or plates or the like in which a surface of such a plate is first ground with sand of progressively increasing fineness applied with hard tools and then polished with rouge under relatively soft tools, the step of smoothing said surface after grinding and before polishing by rubbing a mixture of rouge and pumice in proportions of between 40 and 66 parts of rouge by weight to 165 parts of pumice of a grade having substantially the following per cent of particles of the indicated fineness between sieves:

| Sieve No. | Per Cent Between Sieves |
|-----------|-------------------------|
| 42        | N                       |
| 48        | 5P                      |
| 60        | FP                      |
| 65        | T                       |
| 80        | 0.4                     |
| 100       | 9.8                     |
| 150       | 30.0                    |
| 200       | 35.0                    |
| 250       | 11.1                    |
| +325      | 7.5                     |
| -325      | 6.2                     |

by weight in water to which copperas has been added to give a reading of between 0.4° and 1.0° on the Baumé scale over said surfaces with compressible tools.

11. In a method of surfacing glass sheets or plates or the like in which a surface of such a plate is first ground with sand of progressively increasing fineness applied with hard tools and then polished with rouge under relatively soft tools, the step of smoothing said surface after grinding and before polishing by rubbing a mixture of rouge and pumice in a liquid carrier over said surface with compressible tools in proportions of substantially 50 parts of rouge by weight to 165 parts of pumice of a grade having substantially the following percent of particles of the indicated fineness between sieves:

| Sieve No. | Per Cent Between Sieves |
|-----------|-------------------------|
| 42        | N                       |
| 48        | 12P+                    |
| 60        | FP                      |
| 65        | 2.7                     |
| 80        | 9.6                     |
| 100       | 17.4                    |
| 150       | 26.1                    |
| 200       | 27.5                    |
| 250       | 8.2                     |
| +325      | 5.5                     |
| -325      | 3.0                     |

60 by weight in water to which copperas has been added to give a reading of substantially 0.6° on the Baumé scale over said surface with compressible tools.

65 12. In a method of surfacing glass sheets or plates or the like in which a surface of such a plate is first ground with sand of progressively increasing fineness applied with hard tools and then polished with rouge under relatively soft tools, the step of smoothing said surface after grinding and before polishing by rubbing a mixture of rouge and pumice in a liquid carrier over said surface with compressible tools in proportions of substantially 50 parts of rouge by weight to 165 parts of pumice of a grade having substantially

the following percent of particles of the indicated fineness between sieves.

| Sieve No. | Per Cent Between Sieves |
|-----------|-------------------------|
| 42        |                         |
| 48        | N                       |
| 60        | 4P                      |
| 65        | VFP                     |
| 80        | 0.1                     |
| 100       | 14.0                    |
| 150       | 42.7                    |
| 200       | 30.8                    |
| 250       | 2.9                     |
| +325      | 5.5                     |
| -325      | 4.0                     |

by weight in water to which copperas has been added to give a reading of substantially 0.6° on the Baumé scale over said surface with compressible tools.

13. In a method of surfacing glass sheets or plates or the like in which a surface of such a plate is first ground with sand of progressively increasing fineness applied with hard tools and then polished with rouge under relatively soft tools, the step of smoothing said surface after grinding and before polishing by rubbing a mixture of rouge and pumice in a liquid carrier over said surface with compressible tools in proportions of substantially 50 parts rouge by weight to 165 parts of pumice between grades characterized by having substantially the following per cents of particles of the indicated fineness between sieves:

| Sieve No. | Per Cents Between Sieves |
|-----------|--------------------------|
| 42        |                          |
| 48        | N                        |
| 60        | 4P                       |
| 65        | VFP                      |
| 80        | 0.1                      |
| 100       | 14.0                     |
| 150       | 42.7                     |
| 200       | 30.8                     |
| 250       | 2.9                      |
| +325      | 5.5                      |
| -325      | 4.0                      |

by weight in water to which copperas has been added to give a reading of substantially 0.6° on

the Baumé scale over said surface with compressible tools.

14. In a method of surfacing glass sheets or plates or the like, the step of smoothing a surface of such a plate by rubbing a mixture of rouge and pumice in proportions of between 40 and 66 parts of rouge by weight to 165 parts of pumice between grades characterized by having substantially the following per cents of particles of

10 the indicated fineness between sieves:

| Sieve No. | Per Cents Between Sieves |
|-----------|--------------------------|
| 42        |                          |
| 48        | N                        |
| 60        | 4P                       |
| 65        | VFP                      |
| 80        | 0.1                      |
| 100       | 14.0                     |
| 150       | 42.7                     |
| 200       | 30.8                     |
| 250       | 2.9                      |
| +325      | 5.5                      |
| -325      | 4.0                      |

15

20

30

25

35

40

45

by weight in water to which copperas has been added to give a reading between 0.4° and 1.0° on the Baumé scale over said surface with compressible tools.

GEORGE E. RICKNER.  
OSCAR F. KOENIG.

#### REFERENCES CITED

The following references are of record in the file of this patent:

#### UNITED STATES PATENTS

| Number    | Name     | Date          |
|-----------|----------|---------------|
| 538,803   | Wefers   | May 7, 1895   |
| 1,231,307 | Spellman | June 26, 1917 |
| 1,373,532 | Showers  | Apr. 5, 1921  |
| 1,996,369 | Ely      | Apr. 2, 1935  |
| 2,000,240 | Long     | May 7, 1935   |
| 2,023,275 | Long     | Dec. 3, 1935  |
| 2,309,819 | Benner   | Feb. 2, 1943  |

#### FOREIGN PATENTS

| Number  | Country | Date           |
|---------|---------|----------------|
| 511,098 | France  | Sept. 18, 1920 |